

# UNITED STATES PATENT OFFICE.

WALTER W. RICHARDS, OF WILMINGTON, DELAWARE, ASSIGNOR TO E. I. DU PONT DE NEMOURS POWDER COMPANY, OF WILMINGTON, DELAWARE, A CORPORATION OF NEW JERSEY.

## ARTIFICIAL LEATHER AND PROCESS OF PRODUCING THE SAME.

1,270,055.

Specification of Letters Patent. Patented June 18, 1918.

No Drawing.

Application filed November 16, 1912. Serial No. 731,653.

To all whom it may concern:

Be it known that I, WALTER W. RICHARDS, of Wilmington, in the county of Newcastle, and in the State of Delaware, have invented 5 a certain new and useful Improvement in Artificial Leather and Processes of Producing the Same; and do hereby declare that the following is a full, clear, and exact description thereof.

10 My invention relates particularly to a manufactured article having the characteristics of real leather, and to the process of making the same.

Artificial leather is ordinarily made by 15 coating a woven fabric with a solution of pyroxylin in a volatile solvent, the solution carrying some coloring matter and non-volatile oil. When artificial leather is made in this manner, the volatile solvent evaporates, 20 leaving behind the oil. In the actual production of the artificial leather, however, traces of the volatile solvent usually remain for a considerable period of time and thereby impart to it an odor which not only indicates 25 that the product is not real leather, but which is also at times disagreeable. Furthermore, the non-volatile oil which is retained in the finished product is subject to changes in composition which oftentimes result 30 in the production of compounds having an odor which is disadvantageous for the same reasons as in the case of the traces of solvent remaining in the finished product.

The object of my invention is to produce 35 an artificial leather which will not only have the appearance and strength of real leather, but will also have the same odor as real leather. An artificial leather of this kind will therefore seem to be, in all respects, the same as leather itself. My object is, furthermore, to provide constituents which will 40 counteract the effects of the solvent and oil retained in the pyroxylin coated fabric, so that the result is to produce the odor of real 45 leather. It will therefore be seen that the actual constituents added to produce this effect are not the same as would be used to obtain merely the odor of real leather, but to produce an odor which, when combined 50 with the odor of the solvent, etc., will give as a result the odor of real leather.

In carrying out my invention I add to the artificial leather certain constituents which not only give to it the requisite odor, but also

have a preservative and softening action 55 which permanently benefits the artificial leather.

My invention is capable of being carried out in many different ways. For the purpose of illustration, however, I will describe 60 it as a product and method of producing the same involving the use of an oily constituent which has an odor and character such that it will accomplish the purposes above indicated. The constituents which I may add 65 are, first, an empyreumatic constituent which will give to the artificial leather the faint burnt or caramelized odor of finished leather; second, an animal oil which will give to it an animal odor; and third, an essential oil or similar substance which acts 70 so as to blend or mask the other odors to some extent. In producing an artificial leather in accordance with my invention, I add to the pyroxylin dissolved in a volatile 75 solvent, a quantity of an empyreumatic distillate or oil, as, for example, oil of Russia leather compound, oil of cade, oil of birch tar, crude or rectified. To this may be added an essential oil as, for example, oil of lavender flowers or oil of bergamot, and in addition may be added an alcoholic animal tincture, as for example, tincture of tonquin grain musk. As an example of the substances which may be added to the solution 80 of pyroxylin, I may add the following: empyreumatic distillate or oil, 90%, essential oil  $\frac{1}{10}$  of 1%, alcoholic animal tincture,  $\frac{1}{10}$  of 85 1%. The fabric is coated with a pyroxylin solution containing these added substances, 90 and is dried in the usual manner. The drying of the coating upon the fabric leaves in the coating composition a sufficient quantity of the added constituents having the desired odors to produce an artificial leather having 95 an odor which cannot be distinguished from that of ordinary leather, and it is found that the artificial leather thus produced retains these constituents for a sufficiently long time 100 to give the artificial leather permanently the odor of real leather.

While I have described my invention above in detail, I wish it to be understood that many changes may be made therein without departing from the spirit of my invention.

I claim:

1. An artificial leather comprising a py-

2. roxylin-coated fabric having the odor of leather and containing an empyreumatic substance.
5. 2. An artificial leather comprising a pyroxylin-coated fabric having the odor of leather and containing musk.
10. 3. An artificial leather comprising a pyroxylin-coated fabric having the odor of leather and containing an animal tincture.
15. 4. An artificial leather comprising a pyroxylin-coated fabric having the odor of leather and containing an empyreumatic substance and an essential oil.
20. 5. An artificial leather comprising a pyroxylin-coated fabric having the odor of leather and containing musk and an essential oil.
6. An artificial leather comprising a pyroxylin-coated fabric having the odor of leather and containing an animal tincture and an essential oil.
25. 7. An artificial leather comprising a pyroxylin-coated fabric having the odor of leather and containing an empyreumatic substance, an animal oil and an essential oil. 25
8. The process which comprises dissolving pyroxylin in a solvent, adding thereto an empyreumatic substance, coating a fabric therewith, and drying the coated fabric.
30. 9. The process which comprises dissolving pyroxylin in a solvent, adding thereto an empyreumatic substance and musk, coating a fabric therewith, and drying the coated fabric.
10. 10. The process which comprises dissolving pyroxylin in a solvent, adding thereto an empyreumatic substance, musk and an essential oil, coating a fabric therewith, and drying the coated fabric.

In testimony that I claim the foregoing I 40 have hereunto set my hand.

WALTER W. RICHARDS.

Witnesses:

L. E. EDGAR,  
HUGH J. MURPHY.